

## UNITED STATES PATENT OFFICE

ARTHUR BORRMANN, OF HAMBURG, GERMANY, ASSIGNOR TO SIEGMUND KOCH, OF HAMBURG, GERMANY

## PROCESS FOR CHEMICALLY IMPREGNATING JUTE SACKS, TENT CLOTH, AND THE LIKE

No Drawing. Application filed March 24, 1930, Serial No. 438,629, and in Germany February 14, 1929.

This invention relates to a novel process for chemically impregnating fabrics, especially jute sacks, tent cloth and the like to render the same waterproof. The new process differs in an advantageous manner from the hitherto known processes of this kind not only in its simplicity and cheapness, but also in the durability and resisting capability of the fabrics treated against 10 climatic and similar influences.

For impregnating such fabrics hitherto caoutchouc or balata were dissolved in benzol or the like by hot method, the impregnated material being subjected to a vulcanization under heat.

Contrary thereto an impregnating liquid is prepared, according to the new process, by cold method from balata, in that balata is dissolved in a mixture consisting of equal 20 parts of carbonic disulphide and trichlorethylene; to which solution filling substances, such as zinc-white, wheat flour, asbestos powder or the like, are added in known manner.

The fabrics treated with this impregnating liquid are immediately ready for use without further treatment after the evaporation of the solvent. The fabrics are then absolutely waterproof and not sensitive to 30 heat or cold, without their losing any of their original suppleness and pliability through the treatment.

Fabrics impregnated in this manner can withstand temperatures up to 100° C., without their usefulness being in any way affected, so that for example jute sacks treated according to the process are suitable in an excellent manner for use in the tropics.

The proportions of the quantities of the 40 several constituents of the impregnating liquid can naturally vary according to the special purposes and requirements, however experiments have shown that, particularly for impregnating jute sacks, tent cloth and similar fabrics, the following composition is in most cases very suitable:

50 parts by weight of carbonic disulphide,  
50 parts by weight of trichlorethylene  
20 parts by weight of wheat flour  
50 20 parts by weight of zinc-white or

40 parts by weight of asbestos powder and

10 parts by weight of balata.

In preparing the composition, the balata is dissolved at an ordinary temperature in 55 a mixture of carbonic disulphide and trichlorethylene. After dissolving completely, the filling substances, wheat flour and zinc-white, are added, whereupon the whole is again thoroughly mixed for about three 60 hours and brought into a suitable reservoir, from which the solution is fed as required through pipe conduits or the like to the vessel to act as the bath.

The jute sacks to be dipped into the bath 65 are preferably stretched tightly over plates of plywood and thus introduced into the bath, in which they are allowed to remain about 1½ minutes. After the sacks have been removed from the bath and roughly 70 drained off, they are dried at ordinary temperature in an exhauster or a similar plant 3 to 5 minutes, when they are ready for use without further treatment.

The process can also be carried out in such 75 a manner that the impregnating mass is applied to the jute sacks by painting machines.

The solvent used can be recovered almost entirely in known manner by evaporation, 80 so that the new impregnating process is very cheap as compared with other processes.

The balata mass is intimately combined with the filling substances employed in the finest uniform distribution in the impregnated fabric and adheres absolutely tightly 85 to the fibres, so that the fabrics have a very great durability without becoming stiff or brittle.

The fabrics treated according to the new 90 process are absolutely impervious to moisture, because the impregnating liquid is not only itself absolutely sterile but any mildew or similar germs present in the fabric are positively destroyed.

Tent cloth and other piece fabrics are 95 treated in a similar manner.

I claim:—

1. The herein described process of waterproofing jute, tent cloth and other fabrics, 100

which consists in dipping the fabric in a stretched state in an impregnating solution formed by dissolving balata in a solvent mixture including a filler for about 1½ minutes, removing the fabric from the solution and permitting any excess deposit to drain therefrom, and thereafter evaporating the solvent of the solution from the mixture remaining with the fabric.

2. The herein described process of water-proofing jute, tent cloth and other fabrics, which consists in saturating the fabric in a stretched condition with an impregnating solution formed by dissolving 10 units of balata in a solvent mixture of 50 units of carbon disulfid and 50 units trichlorethylene and adding a filler, in draining the fabric to permit excess solution to be dislodged therefrom, and subjecting the fabric to an exhauster for vaporizing the solvent of the solution.

In witness whereof, I subscribe my signature.

ARTHUR BORRMANN.

25

30

35

40

45

50

55

60